

## UNITED STATES PATENT OFFICE.

CARL W. VOLNEY, OF BOSTON, ASSIGNOR TO GEORGE M. MOWBRAY, OF  
NORTH ADAMS, MASSACHUSETTS.

## IMPROVEMENT IN EXPLOSIVE COMPOUNDS.

Specification forming part of Letters Patent No. 124,397, dated March 5, 1872.

I, CARL W. VOLNEY, of Boston, Massachusetts, a citizen of the United States, have invented a new and useful Explosive Compound, to be used for blasting, in shells, torpedoes, and for military, naval, or civil engineering purposes, where a powerful and perfectly safe explosive is required, possessing similar explosive properties to nitro-glycerine, but which is incapable of being exploded by concussion or agitation, nor is it liable to spontaneous decomposition; for instance, thrown upon a fire, or red hot coals, it burns with flame and without explosion; placed on a cold anvil and struck with a blacksmith's hammer it does not explode. The common mode of exploding nitro-glycerine, as patented by A. Nobel, will not explode it. The very powerful electric fuse-exploders, patented by G. M. Mowbray, however, are capable of exploding it, in which case there is no tamping or confinement needed.

It may be transported in any vehicle, railroad car or steamboat, absolutely without the possibility of explosion; and in case of fires would only burn like oil.

The above are some of the features which distinguish this compound from nitro-glycerine. Being a homogeneous liquid, at ordinary temperature, when exploded in the manner described, it is wholly converted into gaseous matter, and this distinguishes it from dynamite, dualin, and other mixtures of nitro-glycerine with inert matter.

To enable others skilled in the art to prepare this compound, I will proceed to describe my process.

In the first place I proceed to make nitro-glycerine by adding one part of glycerine to nine parts of a mixture composed of sixty-six parts of sulphuric acid 66° Baumé, and thirty-

three parts of nitric acid 50° Baumé, adopting the usual precautions to avoid overheating; and, when the ingredients have reacted, pouring the mixture into water and thoroughly washing the product. This gives me 1.5 parts of nitro-glycerine. I next prepare in a precisely similar manner what I call nitrotoluol, substituting, however, for the glycerine used in the above-mentioned process, benzole of commerce, the boiling point of which I prefer should be from 110° to 120° Fahrenheit, and for the nitro-sulphuric acid, substituting nitric acid of the specific gravity of 1500°. I now dissolve three parts of the latter compound, which I have termed nitrotoluol in seven parts of the nitro-glycerine, making a homogeneous liquid; this is the explosive compound which I have invented.

Variations of these proportions may be used, but if the compound termed nitrotoluol is used in greater proportion than above specified, I have found in close tunnels, mining levels, or places where the ventilation is imperfect, that the gases given off after the explosion are apt to affect the miners injuriously.

Having thus fully described my new compound, I would state that I am aware that, in the patent granted to A. Nobel, benzole is mentioned as a substance which may be mixed with nitro-glycerine; this I do not claim, but—

What I do claim and desire to secure by Letters Patent, is—

An explosive mixture consisting of nitro-glycerine and nitrotoluol or nitro-benzole, in about the proportions herein described.

CARL W. VOLNEY. [L. S.]

Witnesses:

GEO. M. MOWBRAY,  
JAMES WALLACE.